

# UNITED STATES PATENT OFFICE.

JOSEPH P. MAXFIELD, OF MILLBURN, AND GEORGE O. SMITH, OF EAST ORANGE, NEW JERSEY, ASSIGNEES TO WESTERN ELECTRIC COMPANY, INCORPORATED, OF NEW YORK, N. Y., A CORPORATION OF NEW YORK.

## RESISTANCE MATERIAL AND METHOD OF MANUFACTURING SAME.

1,403,803.

Specification of Letters Patent. Patented Jan. 17, 1922.

No Drawing.

Application filed July 12, 1919. Serial No. 310,440.

To all whom it may concern:

Be it known that we, JOSEPH P. MAXFIELD and GEORGE O. SMITH, citizens of the United States, residing at Millburn, in the county of Essex, State of New Jersey, and at East Orange, in the county of Essex, State of New Jersey, respectively, have invented certain new and useful Improvements in Resistance Materials and Methods of Manufacturing Same, of which the following is a full, clear, concise, and exact description.

This invention relates to resistance materials and more particularly to a granular type of resistance material suitable for telephone transmitters and a process of manufacturing such a material.

To meet satisfactorily the requirements of a resistance material for use in telephone transmitters and similar places, it is of a decided advantage to have the granules light and of substantially globular shape so that they will not pack together and cause unsatisfactory operation of the transmitter itself. In certain types of transmitters, it is also of importance that the carbon particles be made light in order that their inertia may retard the movement of the diaphragm as little as possible.

It is, therefore, the object of the present invention to provide a granular resistance material, particularly for use in telephone transmitters, which is substantially globular in shape, light in weight and has a firm hard surface.

To attain this result and in accordance with a feature of this invention, a resistance material is made by mixing ground carbon particles with a binder in such a way as to give a globular shape, and roasting the mixture to give the desired resistance and surface firmness.

The preferable method of manufacturing this type of resistance material is as follows:

A powdered carbon is obtained by reducing cane sugar to carbon in an open kettle by means of a low flame and then grinding in a ball-mill until the resulting product is fine enough to pass through a 200 mesh sieve.

The binder with which this powder is to be mixed is made by filling a pot approximately one-fourth full with cane sugar and then heating over a low flame, the reduction

being carried to a point where the sugar gives off pungent odors and ceases to rise in the pot. Hot water is then poured in slowly until the mixture has a specific gravity of from 1.27 to 1.33.

The powdered carbon and the caramel are mixed together to produce a thick paste having approximately the consistency of putty. This mixture is then forced through a sieve, the mesh of which is approximately 15% greater than the desired size of the resulting product. For the standard grades of carbon the size of this sieve will range from ten to forty mesh. This increased size of the material as sieved is necessary to provide for the shrinkage of material during the roasting operation.

The mixture, after being sieved, is placed in a rotating or ball-mill (but without the customary steel balls) and is rotated for a period of from twelve hours to three days, after which it is sieved to remove the smaller globules. The product is then dried in an oven at a temperature slightly below the boiling point of water for a period of approximately four hours to remove all water from the binder gradually so as not to form cracks in the carbon globules. It is then placed in crucibles where it is protected from oxidation by means of a covering of carbon which keeps out the air, and the temperature raised slowly so that at the end of a period of two hours a temperature of approximately 300° C. is reached. The temperature is then raised to a temperature of 500° C. during the next hour and then raised rapidly to the final heat desired which is a bright red heat.

The product is allowed to cool and is then placed in a wire cage inside of a tank and all air exhausted. Additional caramel is then inserted under pressure and tends to force itself into the small cavities and pores in the surface of the globules. The container with the carbon globules impregnated with caramel is then placed in a centrifuge to remove all excess caramel and to keep the particles from sticking together. The carbon globules are then placed on drying trays which are maintained at a temperature slightly below boiling for a period of four hours, the grains being stirred at intervals of approximately one-half hour. The product is then heated in crucibles or an

iron retort to a temperature of 600° C. for carbonization of the caramel filler. The operation of filing the globules with a caramel filler which is then carbonized is 5 repeated a number of times, depending upon the strength and hardness required on the surface. For ordinary use, this operation is performed about four times, although for certain grades of carbon it has been found 10 preferable to perform this operation as many as ten times. After the final impregnating operation, the product is heated in crucibles to a final temperature ranging from 1000° to 1400° C. depending upon 15 the desired resistance of the carbon.

The resistance material made by following the above process not only has the advantage of freedom from packing as a result of its substantially spherical shape and 20 its lightness, but it also impedes the motion of light vibrating systems a minimum amount. For detectophones and similar apparatus which must remain sensitive to very weak sounds, it is of importance that this 25 impedance to motion be kept as low as possible. The apparent density of the resistance material made by following in detail the process described is approximately .5 grams per cubic centimeter and slight variations 30 from the specific process described may be made and the apparent density of the product kept within the limits of .4 to .7 grams per cubic centimeter. This light weight, however, does not involve a sacrifice 35 of the wearing quality and permanence of the product. By following the process described and by small changes in the temperature of carbonization of the filler, it is possible to produce carbon globules which are 40 porous at the center but of increasing density toward the outer surface which is comparatively hard and smooth or to produce firm globules of uniform texture throughout.

What is claimed is:

- 45 1. A granular resistance material consisting of carbon granules substantially globular in shape and having an apparent density of approximately .50 grams per cubic centimeter.
- 50 2. A granular resistance material consisting of carbon granules substantially globular in shape, said globules being of increasing density from the center toward the surface.
- 55 3. The method of manufacturing a resistance material which consists in forming

porous globules of resistance material, and then forcing similar material in a plastic state into the surface pores.

4. The method of manufacturing a resistance material which consists in mixing a resistance material with a binder, sieving the mixture, rotating the product to form particles substantially globular in shape, and roasting such globular material to give the 60 desired resistance.

5. The method of manufacturing a resistance material which consists in grinding carbon to a powder of the desired fineness, mixing this powder with a binder to produce 70 a material having approximately the consistency of putty, forcing this mixture through a sieve, rotating the sieved mixture to form globules substantially spherical in shape, roasting the globules, impregnating 75 the globules with a filler, and again roasting the product to produce further carbonization to give the desired resistance.

6. The method of manufacturing a resistance material which consists in grinding 80 carbon to a powder of the desired fineness, mixing this powder with a caramel binder to produce a material having approximately the consistency of putty, forcing this mixture through a sieve, rotating the sieved mixture to form globules substantially spherical in shape, roasting the globules, impregnating the globules with a caramel 85 filler, and again roasting the product to produce further carbonization to give the 90 desired resistance.

7. The method of manufacturing a resistance material which consists in grinding carbon to a powder of the desired fineness, mixing this powder with a caramel binder 95 to produce a material having approximately the consistency of putty, forcing this mixture through a sieve, rotating the sieved mixture to form globules substantially spherical in shape, drying the globules 100 slowly to remove all water, roasting the globules, placing the roasted globules in a tank, exhausting all air from the tank, forcing caramel into the tank under pressure, removing all excess caramel by means 105 of a centrifuge, and again roasting the product to produce further carbonization to give the desired resistance.

In witness whereof, we hereunto subscribe our names this 10th day of July, A. D. 1919. 110

JOSEPH P. MAXFIELD.  
GEORGE O. SMITH.